

Nov. 14, 1944.

L. N. BENT

2,362,878

## EXPLOSIVE

Filed Aug. 20, 1941



LEAVITT N. BENT  
INVENTOR.

BY Cleveland B. Holloman.

## UNITED STATES PATENT OFFICE

2,362,878

## EXPLOSIVE

Leavitt N. Bent, Wilmington, Del., assignor to  
 Hercules Powder Company, Wilmington, Del.,  
 a corporation of Delaware

Application August 20, 1941, Serial No. 407,512

10 Claims. (Cl. 52—11)

This invention relates to improved blasting explosives and more particularly to explosives containing calcium nitrate as an ingredient.

Explosives, such as the commercial dynamites, usually are comprised essentially of mixtures of 5 nitroglycerin or similar liquid explosive nitric esters, one or more oxidizing salts, such as sodium, potassium, or ammonium nitrate, and a carbonaceous or reducing material, such as wood pulp, ground balsa, manioc meal, wood 10 flour, or the like. The inclusion of an oxidizing salt in the dynamite compositions is most important as it affects the strength of the explosive and the oxygen balance of the admixture. It has been long realized that calcium nitrate theoretically would provide certain definite advantages over the sodium, potassium, and ammonium nitrate that are now used. Thus, for 15 example, the oxygen balance of this material is superior to that of sodium nitrate. Further, less energy is absorbed by the calcium nitrate in decomposing to produce a given weight of oxygen. However, calcium nitrate normally exists in the form of the hydrate containing four molecules of water, and this water of crystallization decreases the amount of oxygen available per unit weight, and the amount of energy available in the explosives which contain it as an ingredient.

It is well known that the hydrate of calcium nitrate can readily be dehydrated by melting the hydrate and boiling the resultant solution with the production of a flour-like material having a particle size of about twenty microns. In this finely divided state, the calcium nitrate is extremely hygroscopic and will quickly absorb moisture from the air even when the relative humidity is quite low. It has been proposed in U. S. Patent 1,865,382 to incorporate this finely divided material as an ingredient in dynamite, but such an ingredient tends to desensitize the powder especially when it contains a relatively low percentage of nitroglycerin. In addition, the powder, in order to be useful, must be packed in completely waterproof containers and must be manufactured in an atmosphere of controlled humidity, i. e., air-conditioned buildings.

The object of this invention is the production of blasting explosive compositions of improved strength.

A further object of the invention is the production of dynamites containing calcium nitrate.

A still further object of the invention is the production of calcium nitrate in a granular form suitable for use in blasting explosives.

A further object of the invention is the pro-

duction of a blasting explosive containing granular free-flowing dynamite.

A still further object of the invention is to provide an explosive containing free-flowing calcium nitrate having a screen size greater than about 150 mesh and preferably a material which will be retained on a 100-mesh screen.

Other and further objects of this invention will appear hereinafter.

The objects of the invention have been accomplished by providing calcium nitrate in a granular form which absorbs water vapor very slowly, and which when incorporated with the normal dynamite ingredients, provides a blasting explosive of improved strength. In more particular detail, the invention comprises producing a granular free-flowing calcium nitrate by evaporating a calcium nitrate solution until a pasty mass is obtained containing 90-95% calcium nitrate (anhydrous basis), which mass will convert into a crumbly mass. The crumbly mass is treated by a heating or pulverizing action at a temperature not exceeding 100° C. until there is produced a granular material. This granular material, upon complete cooling, is composed of compact, very hard granules which do not tend to absorb moisture readily. In addition to this method, a granular calcium nitrate also may be prepared by completely evaporating all water of crystallization present in calcium nitrate and then admixing the resultant fine flour-like anhydrous material with a binder and granulating the admixture either by rubbing it through a screen, kneading, or similar operations.

In the manufacture of blasting explosives, such as dynamite, it is preferable for the oxidizing salts used to be in the form of moderately coarse free-flowing granules. For example, the salts used may be held on a 150-mesh screen and preferably held on a 100-mesh screen. It has been found that by preparing the calcium nitrate in accordance with this invention that a granular material which will be held on a 100-mesh screen can be produced and that this type granular material has a much lower rate of moisture absorption than flour-like calcium nitrate. The influence of the particle size of the calcium nitrate on the rate of the moisture pickup is shown in the attached graph. The graph shows the total gain in weight of three samples of coarse material and a sample of anhydrous flour-like material. Each sample was packed in paraffined paper wrappers and exposed for a definite number of days to an atmosphere held at 70° F. and having a relative humid-

ity of 65%. It will be seen that curve 1 is directed to anhydrous flour-like calcium nitrate and that this material picks up moisture quite rapidly but that the granular material of curves 2, 3, and 4, directed to calcium nitrate having a screen size of between 40 and 100-mesh 20 and 40-mesh, and 9 and 20-mesh respectively, absorbs moisture quite slowly.

The granular product which is obtained in accordance with this invention may be used in the formulation of dynamite especially to replace sodium nitrate and such replacement can be made on an approximately 1-1 basis and will produce a dynamite of considerably higher strength than a dynamite containing an equal weight of sodium nitrate. The percentage of calcium nitrate which may be used corresponds to the percentage of sodium nitrate that may be used and in general will be between 5% and 65% of the total weight of the explosives. Calcium nitrate may be the only oxidizing agent in the explosive composition, or it may be mixed with sodium nitrate, ammonium nitrate, ammonium perchlorate, or the like to obtain any particular characteristic which may be desired. The preparation of the dynamite is carried out by the methods which are standard and well known in the explosive art.

In order to show the adaptation of the calcium nitrate of this invention to use as an ingredient in dynamite compositions, the following examples are given. It will be noted from the examples that by substituting calcium nitrate for sodium nitrate an explosive of considerably higher strength is obtained, and further, it will be noted that the examples given cover each of the standard types of dynamite. Therefore, it will be appreciated that the calcium nitrate may be used in any normal dynamite formulations.

Calcium nitrate sample 2 contained 1.5% rosin which acted as a binder and produced the desired granular form.

if compared to explosives containing fine flour-like calcium nitrate. To show this difference the composition and properties of two samples of straight dynamite, one containing granular calcium nitrate and the other containing flour-like calcium nitrate are given below.

TABLE II

|    | Ingredients                          | Per cent | Per cent |
|----|--------------------------------------|----------|----------|
| 10 | Nitroglycerin.....                   | 20.0     | 20.0     |
|    | Calcium nitrate granular.....        | 61.4     | 61.4     |
|    | Calcium nitrate flour-like.....      |          | 61.4     |
| 15 | Carbonaceous material.....           | 18.1     | 18.1     |
|    | Chalk.....                           | 0.5      | 0.5      |
|    | 1/4 x 8 cartridges/50 lbs.....       | 112      | 107      |
|    | Gap propagation sensitiveness:       |          |          |
|    | As manuf. .... inches.....           | 22       | 16       |
|    | After 5 days at 120° F. .... do..... | 14       | 7        |
|    | Detonation rate..... meters/sec..... | 3,300    | 3,200    |

In addition to the preparation of the calcium nitrate by thermal treatment with kneading or by granulating by means of a binder, such as for example, gum arabic, nitrocellulose, rosin or the like, it has also been found desirable to reduce the rate of moisture absorption of the calcium nitrate particles still further by coating the particles with a thin film of a water-impervious mixture. Thus, for example, the granular material may be treated with an admixture of rosin, paraffin, and petrolatum having an approximate composition of 40, 10, and 40 respectively by adding from 0.5-3% of the rosin-paraffin-petrolatum mixture to the granular calcium nitrate, and agitating the granules by means of a plow, such as is used in a crystallizing pan or by means of a grainer, such as a revolving drum or other suitable method until each individual granule of calcium nitrate has coated thereupon a very thin film of the water-impervious admixture. The effect of the coating on water absorption is shown in Table III.

TABLE I

|                                                                | Example               |       |                               |       |                       |       |                      |       |
|----------------------------------------------------------------|-----------------------|-------|-------------------------------|-------|-----------------------|-------|----------------------|-------|
|                                                                | 1                     |       | 2                             |       | 3                     |       | 4                    |       |
|                                                                | 20% straight dynamite |       | 20% ammonium nitrate dynamite |       | 40% straight dynamite |       | 20% gelatin dynamite |       |
|                                                                | A                     | B     | A                             | B     | A                     | B     | A                    | B     |
| Nitroglycerin.....                                             | 20.0                  | 20.0  | 11.0                          | 11.0  | 39.9                  | 39.9  | 20.0                 | 20.0  |
| Nitrocellulose.....                                            |                       |       | 13.5                          | 13.5  | 6.1                   | 6.1   | 0.2                  | 0.2   |
| Ammonium nitrate.....                                          |                       |       | 55.3                          | 55.3  | 47.8                  | 47.8  |                      |       |
| Sodium nitrate.....                                            | 61.4                  |       | 61.4                          |       | 55.3                  |       | 60.3                 | 60.3  |
| Calcium nitrate <sup>1</sup> .....                             |                       |       |                               |       |                       |       |                      |       |
| Calcium nitrate <sup>2</sup> .....                             |                       |       |                               |       |                       |       |                      |       |
| Wood flour or other carbonaceous material.....                 | 18.1                  | 18.1  | 15.7                          | 15.7  | 11.3                  | 11.3  | 14.5                 | 14.5  |
| Sulfur.....                                                    |                       |       | 4.0                           | 4.0   |                       |       | 4.0                  | 4.0   |
| Chalk.....                                                     | 0.5                   | 0.5   | 0.5                           | 0.5   | 1.0                   | 1.0   | 1.0                  | 1.0   |
| 1/4 x 8" cartridges/50 lbs.....                                | 100.0                 | 100.0 | 100.0                         | 100.0 | 100.0                 | 100.0 | 100.0                | 100.0 |
| Wt. strength (determined with ballistic mortar), per cent..... | 103                   | 112   | 106                           | 110   | 93                    | 104   | 81                   | 88    |
| Gap propagation sensitiveness..... inches.....                 | 20                    | 33    | 20                            | 32    | 40                    | 48    | 20                   | 35    |
|                                                                | 26                    | 22    |                               |       | 38                    | 40    | 4                    | 6     |

<sup>1</sup> Screen analysis of this sample: thru 20 on 40 mesh—22%, thru 40 on 60—12%, thru 60 mesh—60%.

<sup>2</sup> Screen analysis of this sample: thru 20 on 40 mesh—32%, thru 40 on 60—23%, thru 60 mesh—46%.

From the above table it will be observed that the calcium nitrate dynamite formulations show materially higher strength than those containing sodium nitrate. The strengths were determined with a standard ballistic mortar and are expressed in terms of the equivalent straight nitroglycerin dynamite.

The use of the granular calcium nitrate of this invention produces explosives which are of improved quality especially in regard to sensitivity

TABLE III  
Moisture absorption in open dish at 79.5% relative humidity and 25° C.—Effect of coating

|                                                      | 1 day    | 2 days   |
|------------------------------------------------------|----------|----------|
|                                                      | Per cent | Per cent |
| Calcium nitrate, granular, uncoated.....             | 10       | 20       |
| Calcium nitrate, granular, coated <sup>1</sup> ..... | 1.8      | 6        |

With 0.7% of a 40:10:40 mixture of rosin, paraffin, and petrolatum.

This application of water-impervious coatings while highly desirable, and while giving a more water-resistant dynamite, is not essential since the granules of calcium nitrate are in themselves somewhat water resistant, and when used in dynamite formulations, produce dynamites that do not set into hard sticks or become insensitive due to water absorption for long periods of time. Other resin and waxy substances may be used as the coating, if desirable.

As previously indicated, the calcium nitrate may be used for the formulation of all types of dynamite in admixture with a wide variety of commonly used ingredients. The calcium nitrate dynamite produced in accordance with this invention may be used for all of the various purposes to which explosives are generally put and such dynamite formulations will be found extremely efficient. By virtue of the use of calcium nitrate in explosive formulation, the quantity of dynamite required may be reduced since the calcium nitrate content increases the weight strength of the explosive. Further, by the use of granular calcium nitrate in dynamite formulations in accordance with this invention, desirable cartridge count may be obtained and various bulk and weight strengths produced in explosive compositions which may otherwise be difficult to obtain with sodium nitrate.

What I claim and desire to protect by Letters Patent is:

1. A blasting explosive comprising an admixture containing a liquid explosive nitric ester, a carbonaceous material, and calcium nitrate, said calcium nitrate characterized by being granular, free-flowing particles of a size that substantially all particles will be retained on a 100-mesh screen.
2. A blasting explosive comprising in admixture a liquid explosive nitric ester and calcium nitrate, said calcium nitrate being characterized by a granular, free-flowing form and having a screen size such that all particles are retained on a 100-mesh screen.
3. A blasting explosive comprising in admixture nitroglycerin, a carbonaceous material, and granular free-flowing calcium nitrate, characterized by a screen size between about 9 and 40-mesh.

4. A blasting explosive comprising in admixture a liquid explosive nitric ester, a carbonaceous material, and a granular free-flowing calcium nitrate having a screen size between about 9 and 40-mesh whereby the rate of water absorption of said calcium nitrate at 70° F. and 65% relative humidity is not more than .1% by weight per day.
5. A dynamite composition comprising about 10 20% nitroglycerin, 18% carbonaceous material, 60% calcium nitrate and .5% antacid, said calcium nitrate being characterized by a granular free-flowing form and a screen size of between 9 and 40-mesh.
- 15 6. A dynamite composition comprising nitroglycerin about 11%, ammonium nitrate about 13%, calcium nitrate about 55%, carbonaceous material about 15%, and antacid about .5%, said calcium nitrate being characterized by a granular free-flowing form and having a screen size between about 9 and about 40-mesh.
- 20 7. A blasting explosive comprising an admixture containing a liquid explosive nitric ester, a carbonaceous material, and coated calcium nitrate, said calcium nitrate having a water-impermeable coating on the surface and characterized by being granular, free-flowing particles of a size that substantially all particles will be retained on a 100-mesh screen.
- 25 8. A blasting explosive comprising in admixture nitroglycerin, a carbonaceous material, and granular free-flowing calcium nitrate coated with a water-impermeable material, and characterized by a screen size between about 9 and 40-mesh.
- 30 9. A blasting explosive comprising in admixture nitroglycerin, a carbonaceous material, and granular free-flowing calcium nitrate coated with a thin film comprising an admixture of a resin and a waxy substance, and characterized by a screen size between about 9 and 40-mesh.
- 35 10. A blasting explosive comprising in admixture nitroglycerin, a carbonaceous material, and granular free-flowing calcium nitrate coated with a thin film comprising an admixture of rosin, paraffin and petrolatum, and characterized by a screen size between about 9 and 40-mesh.
- 40
- 45

LEAVITT N. BENT.